

## UNITED STATES PATENT OFFICE.

WILLIAM LEWIS, OF VANCOUVER, BRITISH COLUMBIA, CANADA.

## DEINKING SOLUTION.

No Drawing. Application filed February 27, 1928, Serial No. 257,541, and in Canada December 12, 1927.

My invention relates to improvements in de-inking solutions, the objects of which are to provide means which will dissolve printer's ink and the like on newspaper and other stock and so neutralize the fatty substances in the ink so as to enable it to be readily washed from the stock that the said stock may be re-used in the formation of paper or other paper products.

10 While many solutions have been compounded for this purpose, their use has entailed much labour and the solution and paper treated has to be subjected for extended periods of agitation at relatively high temperatures to the end that the process of reclaiming the de-inked pulp cost more than the value of the pulp. With the use of the solution hereinafter described, the paper, reduced to pulp form, is treated at ordinary water 15 temperature and the ink removed therefrom with such celerity as to render the process very economical.

The solution is composed of certain ingredients which will obviously vary in quantity 20 according to the paper stock to be de-inked and the components or quality of the ink used thereon. Generally on a common paper stock such as newsprint, a much weaker solution is required than for highly calendered papers.

25 For the de-inking of newsprint, I mix five parts of water glass consisting of sodium silicate, potassium silicate or both, with two parts of caustic soda or concentrated lye and one part of Pearline washing powder in about five thousand parts of water. The chemical 30 composition of Pearline is as follows:

|                                 | Per cent. |
|---------------------------------|-----------|
| Moisture ( $H_2O$ )             | 44.90     |
| Sodium carbonate ( $Na_2CO_3$ ) | 32.50     |
| 40 Soap powder (dry)            | 21.90     |
| Sodium peroxide                 | .70       |

45 I then immerse the printed paper therein, macerating it and keeping it alternately under agitation and squeezing it between suitable surfaces to express the solution and its ink content therefrom, subsequently repeating the process as may be required to entirely remove the ink.

50 I have also found that very satisfactory results can be obtained by the use of a solution

containing waterglass alone, or without the addition of the other ingredients hereinbefore referred to.

The action of the solution upon the macerated stock liberates the ink, which being of 55 lesser specific gravity than the solution floats readily to the surface and may be run off as it accumulates, if desired.

The paper so treated can be entirely freed of ink by successive immersions in this solution without heating and I have found that clean commercial pulp can be obtained from ordinary printed newsprint in from two to 60 four minutes.

It will thus be seen that I have invented an 65 extremely simple solution and method of de-inking printed paper, which is both economical and effective.

What I claim as my invention is:

1. The method of de-inking printed paper 70 stock which consists of saturating the paper in a solution of washing powder, lye, water-glass and water, and subsequently expressing the solution from the resulting pulp.

2. A de-inking solution consisting substan- 75 tially of five parts of water glass, two parts of caustic soda, one part of Pearline and water in suitable proportion.

Dated at Vancouver, B. C., this 17th day of February, 1928.

80 WILLIAM LEWIS. 85

85

90

95

100